

Nov. 1, 1927.

1,647,950

R. F. BACON ET AL

COLLAR AND CUFF AND METHOD OF MAKING THE SAME

Original Filed April 1, 1922

Fig:1.



Fig:2.



Fig:3.



Fig:4.



Fig:5.



Inventors  
Raymond F. Bacon  
Cleo H. Kidwell

By their Attorney

Philip D. Reed

Patented Nov. 1, 1927.

1,647,950

## UNITED STATES PATENT OFFICE.

RAYMOND F. BACON, OF NEW YORK, AND CLEO H. KIDWELL, OF ST. GEORGE, NEW YORK, ASSIGNEES, BY MESNE ASSIGNMENTS, TO VAN HEUSEN PRODUCTS, INC., A CORPORATION OF DELAWARE.

### COLLAR AND CUFF AND METHOD OF MAKING THE SAME.

Original application filed April 1, 1922, Serial No. 548,604, and in Canada May 27, 1922. Divided and this application filed March 22, 1923. Serial No. 626,845.

The present invention relates to improvements in collars and cuffs and methods of making the same, and more particularly to collars and cuffs of the "semi-stiff" type, such, for example, as those made of multiple ply interwoven fabric. We do not herein claim collars, cuffs or other articles of apparel having therein a chemically produced natural fold line, inasmuch as such collars and cuffs constitute the subject matter of another application filed by us April 1, 1922, Serial #548,604, upon which a patent was granted April 15, 1924, Patent No. 1,490,081, and of which the present application is a division.

One of the objects of the invention is to provide in such cuffs of the "French" or turn-over variety and in such collars of the folding or turn-down variety and also of the stand-up variety having turn-down tips or wings, permanent fold lines along which the cuffs and collars will tend to fold without altering the weave of the fabric at such lines.

Heretofore, collars and cuffs of the character referred to have in many instances been provided with fold portions of increased flexibility, the said fold portion being produced in the weaving of the fabric, for example, by omitting certain of the warp threads and the interweave or binder threads along this flexible fold portion. In weaving fabrics in this manner for the manufacture of collars the fabric itself and the weakened fold portions have, in some instances, been given a curvilinear contour by drawing the fabric from the loom over conical take-up rolls, as fully set forth and described in patents to Morgan Nos. 1,254,339 and 40 1,254,340.

According to the present invention we produce a permanent natural fold of any desired contour and location after the fabric has been woven, and either before or after the collar or cuff has been cut out. The fabric itself may be woven either in curvilinear or straight form.

Broadly stated, our invention comprises, first, subjecting the fabric along the line at which the natural fold is to be produced, to the action of an acid, folding and press-

ing the fabric along the said natural fold line, and then washing out the acid. We have found that by utilizing a very dilute acid solution of the proper degree of dilution and by subjecting the fabric to its action for the proper length of time at a proper temperature, and pressing the fabric preferably when folded in the desired position, the fabric so treated will be provided with a natural and permanent fold line. That is to say, the fabric when folded will always tend to fold along the line thus treated.

The strength and the particular kind of acid used, and the duration of the acid treatment vary with the particular material treated. So also the particular method of subjecting the material to the acid may vary widely. Accordingly we shall not endeavor herein to describe all of the ways in which our invention may be practiced. But in order that those skilled in the art may understand the invention fully and may apply it to any desired material, we will, for purposes of illustration merely, and not with the intention of limiting the scope of the invention in any respect, describe one way in which we have applied the invention to one type of fabric with excellent results.

The fabric of which the collars and cuffs of "semi-stiff" type are made may be, for example, a multiple ply interwoven fabric with or without an intermediate filler thread layer or layers. One suitable weave of a fabric of this type is illustrated and described in the hereinbefore referred to patents to Morgan Nos. 1,254,339 and 1,254,340. Fabrics of this kind possess a considerable degree of inherent stiffness and set, so that collars and cuffs made therefrom are substantially free from wrinkling and flimsiness and do not require the use of starch or other stiffening material in the laundering operation.

The fabric whose treatment we are about to describe is a two-ply interwoven fabric having an intermediate layer of warp filler threads. For this particular fabric we have found that sulphuric acid of a strength of .5% by weight gives excellent results. The acid may be applied to the fabric along

the desired line of fold of a width of say  $\frac{1}{4}$ ". The fabric may then be folded along the line of acid treatment and subjected to a temperature of about 100° C. and a pressure comparable to that used in an ordinary commercial ironing machine. After this treatment has been carried out the fabric is washed with water and subsequently, if desired, with an alkaline solution, although we do not consider the alkaline bath to be essential. In carrying out this process the fabric may be ironed flat, after the acid has been applied, and then after washing out the acid, it may be folded along the line of acid treatment and pressed, although we prefer the method described above, namely, pressing the fabric while in folded condition during the acid treatment.

The pressure and heat treatment to which the fabric is subjected after the acid has been applied, if carried on for too long a period will tend to char and discolor the fabric. We have found that about one minute is a satisfactory time, although a good fold portion may be obtained without discoloration by treating the fabric for only a few seconds up to about ten minutes.

The invention will be further described in connection with the accompanying drawings 30 illustrative of certain embodiments thereof, in which

Fig. 1 is a perspective view of a folding or turn-down collar embodying the invention; Fig. 2 is a plan view of the collar of Fig. 35 1 unfolded;

Fig. 3 is a perspective view of a stand-up collar with turn-down wings;

Fig. 4 is a plan view of the collar of Fig. 3 laid out flat; and

Fig. 5 shows a cuff of the character that may be made according to our invention.

Referring to the drawings, Figs. 1 and 2 illustrate a collar of the folding or turn-down type, the folding or turn-down portion 45 of which is indicated by the reference numeral 1, the neckband portion by 2 and the natural fold portion by 3. In the example here shown the fold is curvilinear. The said natural fold portion 3 is produced by treating the fabric along the line at which the collar is to fold with a dilute solution of sulphuric acid, folding the fabric along that line, either before or after the application of the acid, subjecting it to the action of heat 50 and pressure while so folded, and thereafter washing out the acid with water or with an alkaline solution or both. The treatment as above described may be made after the fabric has been cut up into collar blanks as shown

in Fig. 2, or the said treatment may be made at any other time after the fabric has been woven that may be deemed advantageous or advisable. It will be obvious that a fold line of any degree of curvature may be obtained either on a straight woven fabric

or on a fabric having a curvilinear contour, by varying as desired the line of application of the acid solution.

Figs. 3 and 4 illustrate a collar of the stand-up type having turn-down tips or wings, the stand-up or band portion of the collar being indicated by reference numeral 4, the turn-down wing portion by 5, and the fold lines of the wing portions by 6. The fold portions 6 along which the wings 5 fold may be produced as set forth above by treating the said lines 6 with a dilute acid solution and then ironing the folded fabric. During the pressing or ironing operation the wings 5 may advantageously be held in the same position with respect to the band portion as the said wings will take in the finished collar, although we do not intend to limit ourselves to any particular position or positions at which the wings shall be held. 85

The cuff of Fig. 5 is of the turn-over or "French" type and its fold line 7 is produced in the manner above described.

It will be understood that the pressure to which the folded fabric is subjected may vary widely, depending on the sharpness or acuteness of the fold portion that is desired. Also the temperature may vary, the effect in general being that the lower the temperature the longer the fabric should be subjected to 95 the action of the acid.

In the above specification and in certain of the appended claims we have employed the term "semi-stiff" as descriptive of the general type of collar or cuff to which this invention refers. By this term we do not mean to define any particular degree of stiffness; but we use it in a broad sense, as including all collars and cuffs which, in their unstarched condition, possess greater inherent stiffness than an ordinary unstarched "soft collar" or "soft cuff" such, for example, as those made from materials of the character used in making negligee shirts. 105

Also, we speak of the natural fold produced by the method described as being "permanent." This term is used in a relative sense only and is intended to cover any natural fold which retains its effectiveness after a succession of launderings. 110

The terms and expressions which we have employed are used as terms of description and not of limitations, and we have no intention, in the use of such terms and expressions of excluding any equivalents of the features shown and described, or portions thereof, but recognize that various modifications are possible within the scope of the invention claimed. 120

What we claim is:

1. In the manufacture of fabric collars or cuffs, the method of producing a natural fold line therein which consists in treating the fabric on the desired line of fold with a dilute solution of sulphuric acid, folding the 130

fabric along said line, pressing it while so folded, and then washing out the acid.

2. In the manufacture of collars or cuffs of semi-stiff fabric, the method of producing
- 5 a natural fold line therein which consists in treating said fabric on the desired line of fold with a solution of about .5% by weight

of sulphuric acid, folding the fabric along said line, pressing it while so folded and while subjected to heat, and then washing 10 out the acid.

RAYMOND F. BACON.  
CLEO H. KIDWELL.